

# UNITED STATES PATENT OFFICE.

ALLAN THOMAS COCKING, OF FOUR OAKS, NEAR BIRMINGHAM, ENGLAND.

## SMOKELESS POWDER.

No. 903,958.

Specification of Letters Patent. Patented Nov. 17, 1908.

Application filed July 23, 1906. Serial No. 327,367.

*To all whom it may concern:*

Be it known that I, ALLAN THOMAS COCKING, a subject of the King of Great Britain and Ireland, and residing at Carhampton 5 House, Four Oaks, near Birmingham, in the county of Warwick, England, have invented certain new and useful Improvements in Smokeless Powders, of which the following is a specification.

10 This invention relates to explosive compounds for use as propellents, and has for its object to produce an explosive which shall have such a regular and uniform rate of combustion as will give the bullet a high velocity

15 with reasonable maximum pressure; which shall produce on combustion a solid residue adapted to act as a lubricant and neutralize acid products of combustion, thus preventing corrosion; and which shall have a moderate

20 temperature of combustion, and so reduce erosion, without materially interfering with the smokeless quality of the powder, and have good chemical stability.

Further objects of the invention are to reduce 25 the volume and luminous character of the flame produced by combustion, to make the explosive compound sufficiently plastic to enable it to be cut when dry without splintering, and to minimize the effects of temperature on the ballistics of the explosive.

The invention consists in the addition to propellant explosives of a salt of the alkali metals, together with a salt of the alkaline earths, whereby after combustion a solid residue 35 due preferably in the form of a carbonate is produced.

The invention further consists in the combination in an explosive for propellant purposes of a carbonate forming salt of an alkali metal and a carbonate forming salt of an alkaline earth together with olive oil or like fixed oil.

The invention further consists in an explosive containing the following ingredients in approximately the proportions given:—

|                |          |        |
|----------------|----------|--------|
| Nitro-glycerin | 30 to 40 | parts. |
| Nitrocellulose | 60 to 50 | parts. |
| Vaseline       | 2.5      | parts. |
| Olive oil      | 2.5      | parts. |

together with a neutral carbonate forming salt of an alkali metal and a neutral carbonate forming salt of an alkaline earth, the proportions of these salts being preferably such as are equivalent to about 0.55 parts of 55 the carbonate of the alkali metal and 2.8 parts of the carbonate of the alkaline earth.

By a carbonate forming salt is meant a salt which when heated to a high temperature decomposes and leaves a residue of carbonate. 60

The invention further consists in the improvements in the manufacture of explosives hereinafter described.

In carrying the invention into effect, for instance, where a potassium salt and a barium salt are used, a mixture consisting of barium tartrate 4 per cent. and potassium tartrate 0.9 per cent. is used. This mixture on combustion in the powder produces 2.8 per cent. of barium carbonate and 0.55 per 70 cent. of potassium carbonate.

The purpose of the addition of the salts of alkali metals and alkaline earths is to produce a solid residue preferably in the form of an alkaline carbonate which will lubricate 75 the gun barrel, and also to neutralize any acid products of combustion which would otherwise cause corrosion, while at the same time producing an explosive which is substantially as smokeless as an explosive in 80 which barium tartrate without potassium tartrate is used and has substantially the lubricating properties of an explosive in which potassium tartrate without barium tartrate is used. For this purpose other carbonate 85 forming salts of the alkali metals and alkaline earths than the tartrates above described may be used, and would produce the same final results or the carbonates themselves may be used in the first instance. It is preferred therefore to use salts such as the tartrates above mentioned which as is well known lower the temperature of the products of combustion. The acetates, citrates, oxalates or bicarbonates may be used for the 90 same purpose; it is especially desirable to use a salt which lowers the combustion temperature as a large proportion of nitroglycerin gives a high temperature, and for small arm ammunition the amount of nitroglyc- 95 erin gives a high temperature, and for small arm ammunition the amount of nitroglyc- 100 erin gives a high temperature, and for small arm ammunition the amount of nitroglyc-

erin should not be less than 30 per cent. to give the necessary plasticity to prevent splintering when the dried powder is cut by the blade of the cartridge loading machine 5 usually employed with explosives of this class.

- The salts of alkali metals and alkaline 10 earths for use as above described are preferably prepared by precipitating them in the form of an impalpable powder from a concentrated aqueous solution by the addition 15 of acetone, alcohol or other liquid which is miscible with water and which is not a solvent for the salt used.
- 15 In order to moderate the speed of combustion of the explosive if desired a small proportion of olive oil or other fixed oil soluble in acetone, alcohol or other solvent used in the incorporation may be used in combination with the salts above mentioned 20 and vaseline may also be used if desired as described in the example hereinafter set out.
- As an example of an explosive in accordance 25 with this invention the following composition may be given:—

|    |                    |          |        |
|----|--------------------|----------|--------|
|    | Nitroglycerin      | 30 to 40 | parts. |
|    | Nitrocellulose     | 60 to 50 | parts. |
|    | Vaseline           | 2.5      | parts. |
| 30 | Olive oil          | 2.5      | parts. |
|    | Potassium tartrate | 0.9      | part.  |
|    | Barium tartrate    | 4.0      | parts. |

- The proportions of nitroglycerin and nitrocellulose may be varied within the above 35 limits, but for an explosive of moderate power the preferred proportion is 35 parts nitroglycerin and 55 parts nitrocellulose.
- The various constituents of the explosive 40 are incorporated in any usual manner, for example, the nitrocellulose is first incorporated with the nitroglycerin; then the vaseline is incorporated with the olive oil and the mixed tartrates amalgamated therewith.
- 45 This latter mixture is then thoroughly incorporated with the first or nitroglycerin nitrocellulose mixture until a homogeneous plastic mass is obtained. To obtain the best results it is preferred to give the explosive compound 50 the shape of strips or flakes of ribbon section with longitudinal ribs. The purpose of the addition of olive oil or like fixed oil soluble in acetone, alcohol or other solvent used in the incorporation, is to reduce the 55 temperature of combustion, while olive oil also has the important property of giving greater chemical stability to the compound. By the use of olive oil in combination with

vaseline the desired moderation in the rate of combustion, chemical stability and reduction in temperature, are obtained. 60

By making up the explosive in the form of strips with projections preferably in the shape of a double headed rail, regular and uniform combustion is obtained, and also 65 high velocity with a reasonable maximum pressure.

The combination of the use of salts which lower the temperature of combustion and the use of olive oil has also the advantage 70 of minimizing the liability of explosives to give higher ballistic effects when subjected to a higher temperature before or at the time of combustion. This result may be further effected by removing the small 75 amount of solvent say 0.5 per cent. which remains in the explosive after it has been dried in the usual drying stove. This may be effected by treating the compound with steam or hot water and thus taking advantage 80 of the affinity of the solvent for water.

It is impossible to limit the application to tartrates or any one particular salt of an alkali metal and an alkaline earth and at the same time adequately cover the invention 85 as there are quite a number of these substances which are useful and the only characteristic which is common to all these salts is that they are formed with acids of high molecular weight and great heat of formation. 90 Similar remarks also apply to the case of the oil as it is not thought necessary to limit this to olive oil or any particular oil and thus exclude other oils which are useful the only characteristic of the various 95 useful oils common to all being that they are oils of high molecular weight and great heat of formation.

Having now particularly described my invention, I declare that what I claim is:— 100

1. A propellant explosive consisting of a homogeneous plastic mixture containing nitrocellulose, nitroglycerin, a tartrate of alkali metal and a tartrate of an alkaline earth, as set forth. 105

2. A propellant explosive consisting of a homogeneous plastic mixture containing nitrocellulose, nitroglycerin, potassium tartrate and barium tartrate, as set forth.

3. A propellant explosive consisting of a homogeneous plastic mixture containing nitrocellulose, nitroglycerin, potassium tartrate, barium tartrate and olive oil, as set forth. 110

4. A propellant explosive consisting of a homogeneous plastic mixture of the follow- 115

ing ingredients in approximately the proportion given.

- 5 Nitroglycerin ----- 30 to 40 parts.  
 Nitrocellulose ----- 60 to 50 parts.  
 Vaseline ----- 2.5 parts.  
 Olive oil ----- 2.5 parts.  
 A carbonate forming neutral salt of an alkali metal equivalent to 0.55 parts of the carbonate of the alkali metal, and  
 10 A carbonate forming neutral salt of an alkaline earth equivalent to 2.8 parts of the carbonate of the alkaline earth.  
 15 5. A propellant explosive consisting of a

homogeneous plastic mixture of the following ingredients in approximately the proportion given.

- |                      |                 |    |
|----------------------|-----------------|----|
| Nitroglycerin -----  | 30 to 40 parts. | 20 |
| Nitrocellulose ----- | 60 to 50 parts. |    |
| Vaseline -----       | 2.5 parts.      |    |
| Olive oil -----      | 2.5 parts.      |    |
| Potassium tartrate   | 0.9 part.       |    |
| Barium tartrate      | 4.0 parts.      | 25 |

In testimony whereof, I affix my signature in presence of two witnesses.

ALLAN THOMAS COCKING.  
 Witnesses:

JOHN MORGAN,  
 HARRY DAVIS.